

Jan. 13, 1959

H. A. DEPEW ET AL  
TREATMENT OF MATERIALS

2,868,673

Filed March 7, 1958

2 Sheets-Sheet 1



Jan. 13, 1959

H. A. DEPEW ET AL

2,868,673

TREATMENT OF MATERIALS

Filed March 7, 1958

2 Sheets-Sheet 2



FIG.2

1

2,868,673

## TREATMENT OF MATERIALS

Harlan A. Depew, Glendale, Patrick D. Quinn, St. Louis, and George R. Waitkins, Des Peres, Mo., assignors to American Zinc, Lead & Smelting Company, St. Louis, Mo., a corporation of Maine

Application March 7, 1958, Serial No. 719,916

20 Claims. (Cl. 117—137)

This invention relates to the treatment of fibrous and porous materials. It has particular application to the treatment of wood and fabric, to render those materials resistant to fire and to the attacks of microorganisms. The term "fabric" is used herein to indicate fibrous sheet materials which may be woven, knitted, felted, laid, or otherwise formed, and to fibers, which may be in the form of yarn, thread, fur, hair, short pieces of stock or the like, which are used to produce these sheet materials. Thus, the term "fabric" includes cloth, (whether of animal fiber, e. g., wool, silk; vegetable fiber, e. g., cotton, linen; mineral fiber, e. g., asbestos; or synthetic fiber, e. g., rayon, nylon) and paper.

While this invention is not limited thereto, it has particular application to cellulosic materials such as wood, and fibers, natural and regenerated.

This application is a continuation as to common subject matter, of applications Serial Nos. 523,383 and 523,386, now abandoned, both filed July 20, 1955.

The need for permanently fire resistant wood is well recognized. The fire code of some cities requires fire resistant treatment of wood used for the interior of buildings, and methods of treatment have been devised which meet these requirements. However, the wood treating processes commonly used heretofore have not produced wood suitable for exterior use, and no commercially accepted method for producing such wood has been developed, in spite of the fact that there is a pressing need for a fire resistant wood for use in ships, railroad trestles, and the exteriors of buildings of all sorts.

One of the materials used heretofore, which renders wood fire resistant and in addition toxic to fungi and termites and yet is non-toxic to warm-blooded animals, is zinc chloride. Zinc chloride has, however, several important undesirable properties. It is readily leached from wood by water. To render wood fire resistant by its use, around four pounds per cubic foot of zinc chloride are required, and when this amount is put into wood, it makes the wood hygroscopic. In humid atmospheres, the water pick up is large. Under these conditions, the zinc chloride dissociates, producing hydrochloric acid that damages the wood severely, so that after a few years the wood has little strength.

Chromates have been added to the zinc chloride in order to make the zinc chloride less corrosive in the treating equipment, and it has been claimed that the addition of the chromates increased the insolubility of the zinc but the evidence does not substantiate the claim.

Since chromium will catalyze combustion, some boric acid and ammonium sulfate are added to the chromated zinc chloride in what is known commercially as the CZC-FR (Fire Resistant) grade, but commercial experience has not justified this composition for wood for exterior service.

A more positive approach to this problem was presented by Ferguson, U. S. Patent No. 1,261,736; Arent, U. S. Patent No. 1,318,524; and Munroe, U. S. Patent No. 1,338,322. They dissolved zinc chloride or a mix-

2

ture of zinc chloride and zinc phosphate in ammonium hydroxide and impregnated the wood with this composition. Then when the ammonia was evaporated they reported the presence of zinc hydroxide and basic compounds that were somewhat insoluble.

We have investigated the methods of Ferguson, Arent and Munroe. In our tests of those methods, zinc chloride was dissolved in aqua ammonia to form a solution containing 14% Zn and 15.7% Cl. Wood was impregnated with the solution and then dried. Fire tube tests on the leached wood showed that around 8 lbs. of zinc, calculated as ZnO, per cubic foot of wood were required to give five tube results below 30%.

| Retention, Lbs./Cu. Ft. ZnO | Days Leaching in Running Water | Percent Fire Tube Loss |            |
|-----------------------------|--------------------------------|------------------------|------------|
|                             |                                | 3 Min. Values          | ASTM Final |
| 8.1                         | 15                             | 17                     | 21         |
| 8.1                         | 30                             | 23                     | 29         |

The performance is satisfactory but the amounts of zinc required are too great to be economically feasible.

In these tests and the tests set out hereafter in connection with the illustrative examples of the process of our invention as applied to wood, the fire tube losses are determined in accordance with ASTM E-69-50-ASTM Standards 1952, part 4, p. 1014. Briefly, in these fire tube tests, a test stick of wood of standard dimensions is suspended vertically within a metal tube or flue, from the beam of a balance which is calibrated in terms of percent of weight of the test stick, rather than in absolute units. That is, the scale of the balance runs from 0% when a standard stick is initially put in place, to 100% when no stick is present. A flame of standard size and intensity is applied to the lower end of the suspended stick. As the stick is consumed by the flame, the percentage loss of weight is indicated directly by a pointer on the balance. This percentage loss is recorded at half minute intervals for four minutes when the applied flame is withdrawn and then continued until the loss of weight for a one minute period does not exceed 1%. Untreated wood will burn to 75-85% loss in less than three minutes. The marginal loss is approximately 40% after four minutes. If more than 40% loss is sustained, the entire stick will be charred. If less than 40% loss is sustained, the flame becomes self-extinguishing and a portion of the stick remains uncharred. A 30% fire tube loss indicates good fire resistance, and 20% is excellent. Except in very exceptional cases, no stick will sustain less than 12% loss. The fire tube loss recorded at the end of three minutes is significant as an indication of the rate of flame spread.

The Pershall Patent No. 2,637,691 represents an advance in the wood treating art over Ferguson, Arent and Munroe. The Pershall process involves preparing basic zinc chloride, dissolving it in aqueous ammonia, and treating wood with the solution. Nevertheless, the Pershall process has several shortcomings. The zinc concentration of the saturated solution is only about 10%, so that it is difficult with many woods to put enough zinc in the wood with one impregnation to give the desired fire resistance. The solution is unstable. On standing, the zinc oxide polymer produced when the basic zinc chloride is dissolved in ammonia breaks down and deposits zinc hydroxide crystals on the walls of the treating container. The deposit in the wood is not uniform. On evaporation of the ammonia, the first precipitate is zinc oxide or zinc hydroxide because of the highly basic nature of the solution. Then very basic zinc chlorides are precipitated, followed by less basic zinc chlorides; then

zinc diamino chloride ( $ZnCl_2 \cdot 2NH_3$ ), and finally, soluble  $NH_4Cl$ . The high pH of the alkaline solution may damage the wood. The adsorbed ammonia tends to increase the chlorine solubility. The presence of ammonium chloride in the wood is not desirable for reasons which are outlined hereafter in connection with Example I.

The impregnation of various fabrics with salts to render them fire resistant, mildew resistant, opaque, or to achieve various other results, is broadly old. Temporary fire resistance has been given by treating cloth with ammonium phosphate, ammonium sulfamate or zinc chloride, but these materials are water soluble and are removed by rinsing. Various phosphorous, chlorine, urea, and resin treatments have been recommended, but the treated cloth has not been sufficiently flame resistant for the purposes to which the fabrics of this invention may be put.

Another treatment that has had commercial success consists of impregnating cloth with a highly acidic solution of titanium and antimony chlorides. After certain intermediate treatment, the acid in the cloth is neutralized with a solution of an alkali such as sodium carbonate. Unfortunately, the acidity of the solution and its tendency to damage the cloth and to corrode the treating equipment limits the usefulness of this treating process. Furthermore, the treated cloth is expensive and may irritate the skin.

It would appear that the teachings of the United States patents to Ferguson, No. 1,261,736; Arent, No. 1,318,524; Munroe, No. 1,338,322 and Pershall, No. 2,637,691, all of which apply to the treatment of wood, might be applied to the treatment of fabric. However, the application of the processes of those references to cloth has produced disappointing results. The ammoniacal solutions required in those processes tend to injure the fabric, the salts are deposited loosely on the surface of the fabric so that they wash out easily, and the fabric dusts badly.

It has even been suggested to deposit salts of tri- and tetra-valent metals in substrates by means of alkylene oxides, but the divalent zinc has been considered too reactive, a suitable process for its use has not heretofore been devised, and the peculiar virtues of its use have remained undiscovered heretofore.

We investigated a process of first treating fabric with zinc chloride and then immersing the impregnated cloth in an alkaline solution in an attempt to deposit basic zinc chloride in the cloth, but this process has proved unsatisfactory. The salts are largely deposited in the liquid and between the fibers of the fabric so that upon being rinsed, the fabric loses its desirable properties.

One of the objects of this invention is to provide a simple, economical, effective process for treating porous and fibrous materials to impregnate them with a basic zinc salt, in such a way that the basic zinc salt is stable and water-insoluble, and resists displacement.

Another object is to provide treated materials which are fire resistant, resistant to the attacks of micro-organisms, termites, and the like, which are resistant to the deteriorating effect of acidic materials, and which are non-hygroscopic and nearly neutral.

In the case of wood, another object is to provide a process which may be used to produce wood of low electrical conductivity, which is readily worked with high speed tools, and is paintable.

Other objects will become apparent to those skilled in the art in the light of the following description and accompanying drawing.

In the drawing, Fig. 1 is a flow diagram of one illustrative embodiment of the process of this invention applied to wood; and Fig. 2 is a flow diagram of one illustrative embodiment of the process of this invention applied to fabric.

In accordance with this invention generally stated, a process is provided by which a basic zinc salt is formed

and deposited in place within the pores of porous material, and in and on the surface of fibers of fibrous materials.

The term "basic zinc salt" is used herein to describe a co-precipitate of zinc hydroxide with a normally water soluble zinc salt. The formula for such a salt may be represented as  $ZnAn.nZn(OH)_2$ , in which  $An$  is the anion of a water soluble zinc salt and  $n$  is a number, the size of which indicates the basicity of the material. The basicity ( $n$ ) is preferably in the neighborhood of 2 to 3, although it may, for certain applications, vary from one quarter to six or seven or more. The pH of the basic zinc salt is less than eight, and in the preferred range of basicities, is about 6.

The process of this invention is a two-step process, wherein the pores of wood or the like or the fibers of fabric or the like are first impregnated with one reactant, and subsequently impregnated with a second reactant, in such a way as to cause, upon the introduction of the second reactant, an initial formation of zinc hydroxide and the subsequent co-precipitation of zinc hydroxide and a water-soluble zinc salt, as a water-insoluble basic zinc salt, in situ.

In treating either wood or fabric, the material to be treated may first be impregnated with a solution of water soluble zinc salt. The solution may be either an aqueous solution or a solution of water soluble zinc salt in an organic solvent such as alcohol. The excess solution is then preferably removed, and the material is subsequently impregnated with a basic material in an amount sufficient to react with the water soluble zinc salt to produce zinc hydroxide, under such conditions as to permit the zinc hydroxide then to combine with the residual water-soluble zinc salt, to form the basic zinc salt.

The term "basic material" is used herein to include alkylene oxides which are acid acceptors, such as ethylene oxide, as well as such bases as ammonium hydroxide, sodium hydroxide, barium hydroxide, ethanol amines and the like. It also includes mixtures of various bases and of bases and acid acceptors. It includes aqueous and organic solutions of bases and of acid acceptors, and the gaseous forms of such acceptors and bases as ethylene oxide and ammonia. It also includes solutions of bases in which zinc salts are dissolved.

In the treatment of fabric, it is necessary that the water soluble zinc salt be added first, and the reactant which produces the zinc hydroxide be added second, and that the basic material be introduced in a medium by which the zinc salt is not leached or dislodged. To this end, the basic material may be introduced as a gas, such as ammonia or an amine of the character of monomethylamine, or a gaseous alkylene oxide, such as ethylene oxide, vaporized propylene oxide, epichlorhydrin, mixed butylene oxides, arylalkyl oxides, cyclo-alkyl oxides and polyepoxy compounds, or in the form of a solution of basic material in an organic solvent in which the water-soluble zinc salt is insoluble.

In the treatment of wood, the wood may first be impregnated with the basic material, and then with the water soluble salt, and such a procedure has certain advantages. In the case of a porous material such as wood, the dislodgment of the first solution is not as much a problem as in the case of the fabric, because the pores serve as little cells, in which the reaction can take place. Thus, the basic materials can include water solutions of ammonium hydroxide, sodium hydroxide, barium hydroxide, and the like, as well as the basic materials listed in connection with the impregnation of fabric.

The precipitated basic zinc salt in the case of fibrous material, is deposited in and on the surface of the fibers in such a way as to strongly resist dislodgment by washing or weathering. The basic zinc salt in the porous material such as wood, is deposited on the walls of the pores, in such a way that the deposit is extremely difficult to dislodge.

Of the water-soluble zinc salts, zinc chloride is pre-

fected. However, the sulfate or nitrate, bromide, iodide or fluoride may be substituted in whole or in part for the chloride. For particular purposes, a part of the chloride, sulfate or nitrate, etc. may be replaced by the phosphates, arsenites, arsenates, borates, and the like. However, the latter anions are used only as additives for particular applications, especially in the treatment of wood.

In the treatment of fabric, various organic addition agents can be added to the fabric during the process of this invention to impart to the fabric such characteristics as softness or a starchy character, water repellance or the like. For example, hydroxyethylcellulose may be dissolved in a zinc chloride solution and will be deposited with the basic zinc chloride when it is precipitated. It gives the cloth a starchy, smooth feel, with increased wash resistance. Examples of other materials which can be dissolved in the zinc chloride solution and which are insolubilized with the deposition of the zinc are polyacrylonitrile and cellulose acetate. An alkyl diketene such as Hercules "Aquapel" may be added to the treating solution as an emulsion, and polyacrylamide can be dissolved in the solution.

In carrying out the process of this invention, as applied to porous materials of which wood will be taken as the example, the wood may be impregnated by pressure or by diffusion. Two general procedures for pressure impregnation of wood are now used. These are what will be referred to hereafter as the empty cell and full cell procedures, respectively.

In the empty cell procedure, the wood is placed in a pressure vessel, commonly a horizontal cylinder, and moderate air pressure is applied. An impregnant solution is then forced into the cylinder and into the wood. Pressure of up to 100-150 pounds per square inch gauge is applied, forcing the impregnant solution deep into the wood. The pressure is then released and the unabsorbed solution is removed from the cylinder. A vacuum is then applied and the residual air in the capillaries of the wood expands, thereby forcing the excess liquid in the pores from the wood. The wood pores are thus covered with a thin film of impregnant. In the two step process of this invention, a considerable volume of open pores is thereby provided for the reception of the second solution.

In the full cell procedure, a high vacuum is applied initially to the pressure vessel containing the wood. An impregnating solution is added to the cylinder and surrounds the wood while the vacuum is maintained. Positive pressure is then applied to force the impregnant into the wood. At the end of the impregnation, the pressure is released. A final vacuum is applied, and the unabsorbed solution is removed from the cylinder. Since the residual air was to a large extent removed from the pores by the initial vacuum, a considerable amount of liquid remains in the pores. However, of the relatively small amount of residual air which was not removed from the pores of the wood by the initial vacuum, some dissolves in the solution during the pressure period. When the pressure is released, this dissolved air comes out of solution in the form of bubbles, causing the wood to bleed. The application of the final vacuum prevents or minimizes bleeding by rapidly removing the solution that would normally run out anyway by virtue of the expansion of the dissolved air.

In the normal practice of the two stage process of this invention, the first solution is added by the empty cell procedure and the impregnation with the second solution follows using the full cell procedure. The chemicals in the two solutions react in the wood and form and deposit a water-insoluble basic zinc salt. The water is then removed from the wood by evaporation.

The empty and full cell procedures can be modified so that no air pressure or a low vacuum is applied before the impregnant solution is introduced. The initial pressure determines the amount of residual air in the capil-

laries and thus is a means for regulating the amount of impregnant solution which remains in the pores.

Many modifications of the operating procedures are possible but in general, the wood is partly filled with the first solution and is then more completely filled with the second solution.

If time is no object, it is unnecessary to use pressure, but diffusion alone may be relied upon. The wood can be fastened down in an open tank containing the first solution. Over a period of time, the air in the pores is displaced by the liquid. The solution is then drawn off and the second solution is added. The chemicals of the second solution diffuse into the wood to react with the chemicals of the first solution to form and deposit water-insoluble basic zinc salts in the wood.

When the diffusion procedure is chosen, the time required will depend upon the size of the piece of wood.

Combinations of full or empty cell procedures and the diffusion procedure may also be used. For example, the pores of the wood may be filled by the full cell process with the first solution. The wood may then be immersed in the second solution to permit the chemicals of the second solution to diffuse into the wood and react with the chemicals of the first solution to form and precipitate the basic zinc salts in the wood.

The following eight examples are illustrative of the process of this invention as applied to wood.

#### EXAMPLE I

30 Fire tube test sticks are placed in a pressure tank and subjected to an air pressure of 50 p. s. i. g. for fifteen minutes. Sufficient of a 33% water solution of zinc chloride (one part of zinc chloride and two parts of water, by weight) is introduced into the pressure tank 35 while the pressure is maintained unchanged, to cover the sticks. Air pressure of approximately 125 p. s. i. g. is then applied to the solution within the tank for one hour. The pressure is then released and the unabsorbed solution withdrawn from the tank. A vacuum of about 40 inches gauge is applied for 5-10 minutes, and any additional free solution is withdrawn from the tank.

An aqueous solution of sodium hydroxide and ammonia, containing 4.7% NaOH, 7.8% NH<sub>3</sub> and the balance water, is then introduced into the pressure tank 45 while the vacuum is maintained. An air pressure of approximately 125 p. s. i. g. is then applied to the basic solution for one hour. The pressure is then released and the unabsorbed solution removed from the cylinder. A vacuum of about 22 inches gauge is applied to remove 50 from the pores any solution which is likely to cause bleeding.

The entire process is carried out at room temperature.

The results are indicated in the following table. The retention of zinc was measured as the difference between the amount of solution introduced into the pressure tank and the amount of unretained solution withdrawn. The actual retention was less, because the residual drawn-off NaOH-NH<sub>3</sub> solution contained 1% of zinc.

|    | Retention, Lbs./Cu. Ft. as ZnO | Percent Fire Tube Losses After 15 Days' Leaching |            |
|----|--------------------------------|--------------------------------------------------|------------|
|    |                                | 3 Min.                                           | ASTM Final |
| 60 | 3.9                            | 25                                               | 34         |
| 65 |                                |                                                  |            |
| 70 |                                |                                                  |            |

The ammonium chloride is preferably kept to a minimum and this has been accomplished, in part, by replacing part of the ammonia with NaOH.

In large amounts, ammonium chloride can interfere with the paintability of the treated wood, cause warping of the wood, and dissolve zinc compounds during leaching. These objections are less applicable to sodium chloride, which is produced when sodium hydroxide is

used. However, the use of sodium hydroxide increases the pH of the treating solution. A mixture of sodium and ammonium hydroxide is, therefore, preferred over a solution of only sodium hydroxide. The use of a strong organic base such as the ethanol amines or their equivalents in place of the sodium hydroxide is more expensive, but technically superior.

A zinc sulfate solution can be used in place of the zinc chloride solution in the process of Example I. To obtain a solution of  $ZnSO_4 \cdot H_2O$  of the same concentration of zinc as the zinc chloride solution, it is necessary to raise the temperature to 50°-60° C. to hold the zinc sulfate in solution. Otherwise, the process may be the same. When zinc sulfate is used in place of zinc chloride, the resultant wood has 10%-15% greater fire loss, but the resultant wood is of better color and holds paint even better than the zinc chloride treated wood.

Mixtures of half zinc chloride and half zinc sulfate give intermediate results.

#### EXAMPLE II

Twenty test sticks, divided into groups of ten, are impregnated at room temperature with 20% zinc chloride solution by the full cell method, the solution being kept under a pressure of about 125 p. s. i. g. for one hour. The unabsorbed impregnant solution is withdrawn from the pressure tank. A vacuum of about 22 inches gauge is applied, and one pound of ethylene oxide gas is admitted to the treating cylinder while the vacuum is maintained. One pound of ethylene oxide is 140% of the theoretical amount required to form  $ZnO$  or  $Zn(OH)_2$  with the retained zinc chloride, based on the following equation:



Owing to the expansion and consequent displacement of impregnant liquid from the pores of the wood during its absorption of the ethylene oxide gas, the wet sticks sustain a weight loss, as shown in the following table:

|                                                    |         |       |
|----------------------------------------------------|---------|-------|
| Dry weight of wood                                 | lbs.    | 3.94  |
| Wet weight of wood                                 | lbs.    | 9.56  |
| Weight of solution absorbed                        | lbs.    | 5.62  |
| Weight of zinc chloride                            | lbs.    | 1.12  |
| Weight of ethylene oxide                           | lb.     | 1.0   |
| Calculated weight of wet sticks and ethylene oxide | lbs.    | 10.56 |
| Actual weight of wet sticks and ethylene oxide     | lbs.    | 9.75  |
| Loss                                               | lb.     | 0.81  |
| Loss                                               | percent | 12.2  |

The following table shows the results obtained by this process:

| Group  | Wt. $ZnCl_2$ Added, Lbs./Cu. Ft. | Wt. $ZnCl_2$ Corrected for Loss | Zinc Calculated as $ZnO$ | Days Leach | Final Fire Tube Loss |
|--------|----------------------------------|---------------------------------|--------------------------|------------|----------------------|
| 1----- | 8.1                              | 7.1                             | 4.1                      | 0          | 30                   |
| 2----- | 8.8                              | 7.7                             | 4.4                      | 15         | 33                   |

Air drying the sticks for 16 hours between the two stages, i. e., between the zinc chloride impregnation and ethylene oxide addition, practically eliminates the salt loss due to the expansion of the zinc chloride solution during gas absorption. The empty cell process may advantageously be used for the zinc chloride impregnation. The ethylene oxide can then be added as a water solution. Since ethylene oxide and water are miscible, an amount of ethylene oxide equal to about 140% of the theoretical requirements as set out above may be used with an amount of water sufficient to immerse the wood. It will be noted that in spite of the 40% excess of ethylene oxide in Example II, the zinc chloride is not converted completely to zinc hydroxide, but rather forms basic zinc chloride. It is believed that as the zinc hydroxide is formed, it

combines with unreacted zinc chloride to precipitate basic zinc chloride which does not react with the ethylene oxide. The amount of the excess of ethylene oxide will determine the basicity of the basic zinc chloride, i. e., the proportion of zinc hydroxide to zinc chloride in the basic zinc chloride. The complete reaction is as follows:



Ammonia gas may be used in place of the ethylene oxide. When ammonia gas is used, it should be added slowly, because the heat of solution and of reaction and the lowered specific gravity of the zinc chloride solution in the wood as the ammonia gas enters the solution tend to cause bleeding of the solution before the basic zinc chloride is formed. The tendency to bleed can be reduced by adding the zinc chloride by the empty cell process and partially drying the wood after it is impregnated with the zinc salt and before the ammonia is added.

There are several advantages in the use of alkylene oxides such as ethylene oxide over the use of ammonia or other similar bases. The wood does not become alkaline. This is true whether the alkylene oxide is introduced as a gas or in water solution.

An additional important advantage of the use of an alkylene oxide arises from the fact that the chlorhydrin produced is non-ionic, i. e., electrically non-conductive and volatile. This permits the wood to be made of low electrical conductance. In order to obtain the lowest electrical conductance, the untreated wood may be leached with water to remove water-soluble salts originally in the wood; dried; impregnated with zinc chloride solution; and treated with an alkylene oxide, either in water solution or as a gas. If desired, it can be dried in a kiln to evaporate any excess of the alkylene oxide and its reaction products, e. g., chlorhydrin. The kiln-treated wood will contain practically pure basic zinc chloride. The wood so treated is of low electrical conductance owing to the absence of water-soluble salts. It has improved dimensional stability.

While ethylene oxide has been used as an example of a suitable alkylene oxide, other alkylene oxides, such as propylene oxide, butylene oxide, epichlorhydrin and styrene oxide may be used. Styrene oxide is less satisfactory than the rest because it is less soluble in water and has a higher boiling point.

#### EXAMPLE III

Test sticks are impregnated with a 33% water solution of zinc chloride by the empty cell procedure as in Example I, and then with a water solution of ammoniacal basic zinc chloride, analyzing 9.3% Zn, 3.9% Cl, and 19.7%  $NH_3$ , by the full cell procedure as in Example I.

| 55 | Retention Calculated as Lbs. $ZnO$ per Cubic Foot of Wood Based on Weight Taken Up | Total                   | Actual Retention Based on Analysis of Wood | Percent Fire Tube Loss After 15 Days' Leaching |            |
|----|------------------------------------------------------------------------------------|-------------------------|--------------------------------------------|------------------------------------------------|------------|
|    |                                                                                    |                         |                                            | 3 Min.                                         | ASTM Final |
| 60 | From $ZnCl_2$                                                                      | From Am. Basic $ZnCl_2$ |                                            | 4.8                                            | 2.1        |
|    |                                                                                    |                         |                                            | 6.9                                            | 5.2        |
|    |                                                                                    |                         |                                            | 16                                             | 24         |

It is evident from columns 3 and 4 that zinc chloride is extracted during the impregnation with the ammoniacal solution. After 15 days' leaching the wood contains 4.5 lbs.  $ZnO$  per cubic foot of wood and 0.9 lb. chlorine per cubic foot of wood.

#### EXAMPLE IV

Test sticks are impregnated with ammoniacal basic zinc chloride to an equivalent  $ZnO$  retention of 1.5 lbs.  $ZnO$  per cubic foot of wood by the empty cell procedure as in Example I, and then after partial drying, with a 33% zinc chloride solution by the full cell procedure

as in Example I. The sticks are leached 15 days and the excess of zinc chloride is removed. Part remains undissolved and combines with the basic zinc chloride. The following table shows the amounts of zinc, calculated as  $ZnO$ , and of chlorine, retained by the wood, and also the fire tube loss, after 15 days' leaching.

| $ZnO$ Lbs./Cu. Ft. Added As—   | Zinc Chloride | Total | Cl Total Lbs./Cu. Ft. | Percent Fire Tube Loss |            |
|--------------------------------|---------------|-------|-----------------------|------------------------|------------|
|                                |               |       |                       | 3 Min.                 | ASTM Final |
| Ammoniacal Basic Zinc Chloride |               | 1.8   | 1.0                   | 2.8                    | 0.4        |
|                                |               |       |                       | 22                     | 37         |

These results are excellent for only 2.8 lbs.  $ZnO$  per cubic foot.

The mechanism of the treatment of this example is thought to be as follows: the zinc chloride reacts with the residual ammonia to form zinc hydroxide, which reacts with more zinc chloride to form basic zinc chloride. Residual zinc oxide, hydroxide, and very basic zinc chloride react with added zinc chloride to form basic zinc chloride with a basicity, for example, of one or two to one.

#### EXAMPLE V

Fifteen test sticks are divided into three groups of five, designated A, B, and C. The sticks of group A are treated with a water solution of chromated zinc chloride containing 30% chromated zinc chloride by weight, by the empty cell procedure as in Example I. The sticks in this group (A) are air dried at 40° C. The sticks of groups B and C are impregnated, together, with the 30% chromated zinc chloride water solution by the same procedure. The sticks of groups B and C are subsequently treated with aqua ammonia containing about 10% ammonia by weight, in an amount of solution sufficient to contain an excess of the quantity of ammonia required to combine with all the chlorine as determined by the amount of chromated zinc chloride retained. The sticks in group B are air dried at 40° C. The sticks in group C are dried at 80° C. The following table indicates the results obtained.

|   | Amounts Used—Lbs./Cu. Ft. Wood                       |                 | Percent Fire Tube Loss After 15 Days' Leaching |            |  |
|---|------------------------------------------------------|-----------------|------------------------------------------------|------------|--|
|   | Chromated Zinc Chloride Calc. as $ZnO$ /Cu. Ft. Wood | NH <sub>3</sub> | 3 Min.                                         | ASTM Final |  |
| A | 5.4                                                  | none            | 25                                             | 66         |  |
| B | 5.2                                                  | 2.5             | 19                                             | 30         |  |
| C | 5.1                                                  | 2.9             | 16                                             | 31         |  |

The results show that the treatment with basic material improves chromated zinc chloride as it does ordinary zinc chloride. However, the fire resistance is probably lowered somewhat by the chromium.

Examples of mixed treating solutions which have given satisfactory results are as follows:

#### EXAMPLE VI

##### 1st solution

|                            | Percent |
|----------------------------|---------|
| $MgCl_2 \cdot 6H_2O$       | 18.0    |
| $NH_4H_2PO_4$              | 5.1     |
| Water (slightly acidified) | 76.9    |

##### 2nd solution

#### AMMONIACAL BASIC ZINC CHLORIDE WATER SOLUTION

|                 |      |
|-----------------|------|
| Zn              | 9.0  |
| Cl              | 3.1  |
| NH <sub>3</sub> | 17.0 |

In the first solution, the water is indicated as being slightly acidified. This is accomplished by adding hydrochloric acid until the pH is approximately 4-5. The acidification is to prevent incipient precipitation of magnesium ammonium phosphate.

#### EXAMPLE VII

##### 1st solution

|                                             | Percent |
|---------------------------------------------|---------|
| 10 $MgCl_2 \cdot 6H_2O$                     | 10      |
| $NH_4H_2PO_4$                               | 2       |
| $ZnCl_2$                                    | 25      |
| Water (slightly acidified as in Example VI) | 63      |

##### 2nd solution

|            | Percent |
|------------|---------|
| 15 Ammonia | 20      |
| Water      | 80      |

#### EXAMPLE VIII

##### 1st solution

|             | Percent |
|-------------|---------|
| 20 $ZnCl_2$ | 30      |
| Water       | 70      |

##### 2nd solution

|                  | Percent |
|------------------|---------|
| 25 $As_2O_3$     | 2       |
| 15% aqua ammonia | 98      |

When wood is treated with zinc chloride solution, and then an alkylene oxide solution is allowed to diffuse into the wood (or the wood with the unremoved zinc chloride solution in it is exposed to an atmosphere of ethylene oxide gas) the difficulties of high pH are avoided. Ethylene oxide is more expensive than the common alkalis and the latter will therefore be preferred in many cases for commercial use.

In commercial practice, for wood for external use, it is desirable to incorporate from four to six pounds of zinc impregnant, calculated as pounds of zinc oxide per cubic foot of wood. The treated wood has the desirable pH of around six which tends to give the wood an even longer life than untreated wood.

The treated wood has high stability to hot water and steam, as a result of which it is particularly adapted to use in cooling towers and wooden hot water tanks.

45 The basic zinc chlorides of this invention affect the wood as if they were deposited along the walls of the pores in the wood. Although the basic zinc chlorides are not very hard, they tend to rigidify the wood, as shown by indentation tests of the wood, but the treated wood

50 saws and handles well on high speed equipment. The zinc of the basic zinc chloride in the wood treated in accordance with the process of this invention neither leaches nor vaporizes from the wood. The treated wood is fire resistant, resistant to fungi, toxic to termites, and 55 repugnant to marine borers. Even barnacles adhere to it to a lesser degree than to untreated wood.

Although this invention as applied to wood is intended primarily for fire resistant wood where considerable amounts of zinc are used, the process is also useful for 60 window sash and all those applications where toxicity to termites is desired and paintability is important. In such cases, one pound per cubic foot and less of zinc calculated as  $ZnO$  is effective. Since basic zinc sulfate treated wood takes paint even better than wood treated with a

65 basic chloride, we prefer it where fire resistance is of secondary importance.

As is evident from the examples, a more highly concentrated solution of zinc salt is generally used in the empty cell process than in the full cell process. For 70 various special applications such as the window sash mentioned above, the concentration used in either process may be varied over wide ranges.

In the case of wood, the introduction of the soluble zinc salt as the second step of the process has the advantage, when the first reactant is an aqueous solution of

a common base, of insuring that there is an excess of the water soluble zinc salt, since, after removal of the free liquid, the amount of base present is limited. This, in turn, insures that the pH of the treated wood will be uniformly low, whereas when the strong base is introduced second, there is some danger of the formation of localized "hot spots" of high pH. This latter danger can be minimized by controlling the conditions of treatment, but it can be eliminated by using the base-soluble salt sequence of steps.

In the treatment of fabric, as has been pointed out above, the fabric is invariably first impregnated with a solution of the water soluble zinc salt.

In comparing the fire resistance of fabrics in the examples which follow, a strip of fabric one inch wide and six inches long is prepared. A Mekker-type gas burner is adjusted to produce a flame about  $1\frac{1}{2}$  inches high. The strip is then suspended from one of its narrow ends so that the lower end just touches the tip of the flame. The cloth is maintained in that position until it has ignited, or, if it will not flame, until the char glows. The piece is rated as follows:

- E—No flaming
- G—Flaming but self-extinguishing
- F—Slow flame spread over all the cloth
- P—Rapid flame spread

Under the conditions of the test, the upper part of the test pieces rated E and G will remain unburned.

The first step in the process of this invention as applied to fabric is the preparation of a solution containing a water-soluble zinc salt, preferably zinc chloride (or bromide, iodide or even fluoride) or zinc sulfate although other salts such as zinc acetate may be used in part. The solution is preferably aqueous, but other solvents such as ethyl alcohol may be used in whole or in part in place of the water.

The fabric to be treated has preferably not been previously treated by any other processes. If the fabric has been sized or otherwise rendered somewhat non-absorbent, the fabric should be rendered absorbent by the removal of the size or other such material.

The fabric is impregnated with the zinc salt solution, either by immersing the fabric in the solution or by spraying or otherwise applying the solution to the fabric. After sufficient of the solution has been absorbed, any free liquid is removed from the fabric by rollers or any other suitable means. The fabric may then be air dried to remove a part of the remaining solvent. The amount of drying required is related to the concentration of the solution. Such air drying is possible, without damage to the fabric, because the solution is not strongly acidic. An alcoholic solution may dry more quickly than an aqueous one. This drying tends to make the treated cloth more resistant to laundering and to minimize any tendency to dusting. While the theory of its operation forms no part of this invention, it is thought that during this drying process, some of the zinc salts migrate from the outside of the fibers to the interior of the fibers.

The second step of the process of this invention as applied to fabric is the supplying, at the site of the water-soluble zinc salt in the fabric, of a reactant, in such a form as to accomplish no substantial leaching or other dislodgement of the water-soluble zinc salt. This second step may be accomplished in any of several different ways. One way is to expose fabric from which the excess of water-soluble zinc salt solution has been removed, to an alkaline gas such as ammonia or an amine, such, for example, as monomethylamine.

Another way is to expose the "damp-dried" cloth to a gaseous alkylene oxide, such as ethylene oxide, or vaporized propylene oxide, epichlorhydrin, mixed butylene oxides, arylalkyl oxides, cyclo-alkyl oxides and polyepoxy compounds.

Another way is to dissolve a basic material such as

ammonia or ethylene oxide in an organic solvent in which the water-soluble zinc salt is insoluble; and spray the "damp-dried" cloth with or dip it in the organic solution.

- 5 Still another way is to dissolve an alkylene oxide such as ethylene oxide, propylene oxide, butylene oxide, epichlorhydrin, styrene oxide or other arylalkyl oxides, cyclo-alkyl oxides and polyepoxy compounds in anhydrous ethyl alcohol along with zinc chloride to form the 10 treating solution and to spray the fabric treated with the solution with moisture. This way is an exception to the soluble salt-basic material sequence, but is consistent with a soluble salt-reactant sequence, since the water is necessary to the reaction, which will not take 15 place without the water.

The third step of the process is the forming and depositing of a basic zinc salt in place in and on the fibers of the fabric. In the case of the initial impregnation of the fabric with an alkylene oxide dissolved in 20 anhydrous ethyl alcohol along with zinc chloride, with the subsequent supplying with moisture, or the exposure of the damp zinc chloride impregnated fabric to alkylene oxide gas, the reaction may be exemplified by the following equation:



When an alkaline gas is used, the reaction may be exemplified by the following equation:



When the third step is complete, the cloth contains the basic zinc salt as an insoluble compound, and in addition will contain soluble inorganic salts or organic compounds such as chlorhydrin. The cloth can be freed of these materials by rinsing in water. The cloth is then dried. Organic materials including chlorhydrin can also be removed by evaporation on heating.

The following examples are illustrative of the process of this invention as applied to fabric.

#### EXAMPLE IX

A piece of five ounce cotton twill was washed to remove any size, and thoroughly dried. It was then 45 soaked in a solution containing 40% zinc chloride and 60% water by weight, for 30 minutes at room temperature. The cloth was removed from the solution and the excess liquid removed from the cloth by a roller-type wringer, at which time the cloth contained solution in the amount of 200% of its dry weight, hereafter referred to as a 200% wet pick-up. The cloth was then dried until the weight was reduced 30-35%. This treatment constitutes the first step in the process.

This cloth was then put in a covered container containing an amount of ethylene oxide equal to 3 mols of ethylene oxide for each mol of zinc chloride contained in the cloth, as calculated from the amount of retained solution. The impregnated cloth was left in the container in contact with the gaseous ethylene oxide for a period of 15 to 20 hours. The cloth was then removed from the jar and air dried at 70° C.

The following table indicates the results obtained:

|                            | Fire resistance | Percent Zn | Percent Cl |
|----------------------------|-----------------|------------|------------|
| Cloth after rinsing.....   | E               | 20.8       | 4.0        |
| Cloth after 1 wash.....    | E               |            |            |
| Cloth after 5 washes.....  | E               |            |            |
| Cloth after 10 washes..... | E-              |            |            |

In each washing cycle the cloth was washed for 10 minutes in a .5% detergent solution at 30° C. in an agitator-type washing machine; rinsed in tap water at 40° C.; dewatered and dried at 70° C. The detergent

used was "Orvus Extra Granules," a Procter and Gamble product. Similar results were obtained with the following detergent:

|                                                                       | Percent |
|-----------------------------------------------------------------------|---------|
| Tall oil-ethylene oxide compounds (Armour's non-ionic Ethofat 242-25) | 29      |
| Sodium tripolyphosphate                                               | 68      |
| Low viscosity carboxymethylcellulose                                  | 3       |
| Total                                                                 | 100     |

The amount of ethylene oxide may be varied over a considerable range, but in general it has been found desirable to have at least one mol of ethylene oxide to one mol of water-soluble zinc salt. The use of more than two mols of ethylene oxide per mol of zinc salt does not appear to improve the product, but tends to speed the process.

It is of interest to note that the addition of copper chloride,  $CuCl_2$ , to either the fabric or wood treating solutions produces, in the ethylene oxide treatment, a green colored fungicidal impregnant.

The treated cloth is dust free, in the sense that no cloud of dust appears, on tearing. It is believed that the ethylene oxide and the chlorhydrin which is formed in the process of reacting with the zinc chloride may react together or with the cellulose to tie the basic zinc chloride formed to the fibers.

The strength of the cloth after the treatment is often as much as 30% or more greater than its strength before treatment.

#### EXAMPLE X

A piece of five ounce cotton twill was treated with zinc chloride solution in the same manner as the cloth in Example I. The cloth, from which the excess liquid was removed as in Example I, was placed on a rotating support in a covered container. The solution retained by the cloth contained a calculated 46 grams of zinc chloride. One hundred grams of ammonia, in the form of 26% aqua ammonia was placed in the bottom of the container. The cloth was kept out of contact with the ammonia solution, but was exposed to the evolved gas. The cloth was exposed to the ammonia gas for 45 minutes, removed from the container, air dried at room temperature, and then further dried at 70° C. to constant dryness. The following table indicates the results obtained:

|                      | Fire resist-<br>ance | Percent<br>Zn | Percent<br>Cl |
|----------------------|----------------------|---------------|---------------|
| Cloth after rinsing  |                      | 22.2          | 5.7           |
| Cloth after 1 wash   | E                    |               |               |
| Cloth after 5 washes | F                    | 17.9          | 1.6           |

Some loose dust appeared before the first wash, but after the first wash the cloth dusted only slightly on tearing.

When using ammonia, the results are improved by adding low concentrations of ammonia over a more extended period of time. It is more difficult to treat fabric uniformly with ammonia than with a slower acting alkylene oxide.

#### EXAMPLE XI

A piece of four ounce viscose rayon cloth was treated with a zinc chloride solution as in the first step of Example IX.

The cloth was then put into a covered container with two mols of ethylene oxide for each mol of zinc chloride.

The ethylene oxide gas was permitted to contact the cloth as in Example IX. The cloth was then removed from the container and, without drying, was rinsed and then dried at 70° C. The fire resistance and zinc and

chlorine content of the cloth are indicated in the following table:

|                      | Fire resist-<br>ance | Percent<br>Zn | Percent<br>Cl |
|----------------------|----------------------|---------------|---------------|
| Cloth after rinsing  | E                    | 24.9          | 5.6           |
| Cloth after 1 wash   | E                    | 20.1          | 2.3           |
| Cloth after 3 washes | F+                   |               |               |

The dusting of the cloth was moderate after rinsing and slight after three washes.

#### EXAMPLE XII

A piece of five ounce cotton twill was treated with the zinc chloride solution of the same strength and in the same manner as in the first step of Example IX, except that the cloth was soaked for 90 minutes.

The cloth was then put into a closed container with two mols of epichlorhydrin per mol of zinc chloride in the cloth. A vacuum was applied to the container. The epichlorhydrin evaporated at the reduced pressure and reacted with the cloth in the container over a period of 48 hours at 25° C. and then for 5 hours at 70° C. The cloth was then air dried, rinsed and dried at 70° C. The cloth was washed at 60° C. The following table indicates the results obtained:

|                      | Fire resist-<br>ance | Percent<br>Zn | Percent<br>Cl |
|----------------------|----------------------|---------------|---------------|
| Cloth after rinse    | E                    | 19.6          | 4.3           |
| Cloth after 1 wash   | E                    |               |               |
| Cloth after 3 washes | G                    | 18.9          | 3.2           |

The various other alkylene oxides which have been suggested heretofore may be used in place of the epichlorhydrin of Example XII.

#### EXAMPLE XIII

Three pieces of five ounce cotton twill identified as A, B and C were washed and dried. Piece A was soaked in a water solution containing 15% zinc chloride. Piece B was soaked in a water solution containing 25% zinc chloride, and piece C was soaked in a water solution containing 35% zinc chloride. The soaking time for each of the pieces was 30 minutes, at room temperature. At the end of 30 minutes, the pieces were removed from their respective solutions and the excess liquid expressed to give a 200% wet pick-up. The pieces were dried at 70° C. for five to ten minutes. The weight losses on drying were 55% for piece A, 50% for piece B, and 40% for piece C. The pieces were put into closed containers with 3 mols of ethylene oxide per mol of zinc chloride. The pieces were allowed to remain in contact with the gaseous ethylene oxide for a period of six hours. They were then removed from the container and dried at 70° C. They were then rinsed in clear water and again dried. The three pieces were washed at 60° C. using a detergent as in Example I. The following table indicates the results obtained:

|                                             | A    | B    | C    |
|---------------------------------------------|------|------|------|
| Concentration of $ZnCl_2$ Solution, Percent | 15.0 | 25.0 | 35.0 |
| Percent Zinc found before rinse             | 11.9 | 16.6 | 19.9 |
| Percent Zinc found after rinse              | 11.6 | 16.7 | 19.4 |
| Percent Cl before rinse                     | 3.3  | 5.0  | 5.9  |
| Percent Cl after rinse                      | 2.5  | 3.3  | 3.6  |
| Fire Resistance after rinse                 | E    | E    | E    |
| Fire Resistance after 1 wash                | F+   | E    | E    |
| Fire Resistance after 3 washes              | F    | G    | E    |

The results shown by the table indicate that within the range of amounts of zinc used in treating pieces A, B and C, the larger the amount of zinc retained, the better the fire resistance of the cloth, and the more permanent the fire resistance with repeated washing.

## 15

The chlorine loss before rinsing appears to be the result of the chlorine's becoming part of an organic molecule which is volatilized.

In carrying out the treatment of cloth using ethylene oxide, the ethylene oxide cost may be reduced by recovering any excess ethylene oxide and reacting any volatilized chlorhydrin with sodium hydroxide or calcium hydroxide to regenerate the ethylene oxide. Other reaction by-products can also be recovered.

## EXAMPLE XIV

Two pieces of five ounce cotton twill, identified as A and B, were treated with a water solution containing 60% zinc chloride to an increase in weight of 140%. The two pieces were then placed in a closed container containing 2 mols of gaseous ethylene oxide per mol of zinc chloride in the cloth, for 18 hours. The pieces were then removed. Piece A was heated to 90-100° C. for 12 hours and then rinsed. Piece B was rinsed without heating. In both cases the basicity of the impregnant in the rinsed cloth was approximately  $ZnCl_2 \cdot 4Zn(OH)_2$ . Approximately 4% of the initial zinc in piece A was dissolved in the rinse water.

Approximately 60% of the chlorine was driven off during the heating of piece A, presumably as chlorhydrin. This accounted for 37% of the added ethylene oxide. Approximately, 8% of the chlorine was leached as chlorhydrin, and 5% as ionic chlorine during the rinsing process. The remaining chlorine was retained by the cloth, so that all of the chlorine was accounted for. Approximately 13% of the added ethylene oxide was not reacted. The ethylene oxide balance with respect to piece A is as follows:

|                         | Percent |
|-------------------------|---------|
| Unreacted               | 13      |
| Volatile as chlorhydrin | 37      |
| Rinsed as chlorhydrin   | 8       |
| Unaccounted             | 42      |
|                         | 100     |

The cloth contained only basic zinc chloride. The unaccounted ethylene oxide must therefore have been volatilized and leached as ethylene glycol or complexes based on this material.

Piece B gave similar results, with the chlorhydrin being leached upon rinsing. All of the zinc and chlorine were accounted for. The unaccounted ethylene oxide was 36%.

The treated cloth showed good fire resistance and hand.

## EXAMPLE XV

Stock was obtained by disintegrating filter paper in water. 36.5 grams of paper pulp was slurried in 2000 grams of a water solution containing 15% zinc chloride. The pulp was then filtered to reform the paper. It was sucked dry and pressed. Two sheets were formed, one approximately  $\frac{1}{16}$  inch thick, the other approximately  $\frac{1}{64}$  inch thick. The sheets of paper were placed in a closed container with 3 mols of ethylene oxide per mol of zinc chloride retained in the paper, for 16 hours, at room temperature. The thick piece of paper showed a fire resistance of E and the thin piece of paper showed a fire resistance of F, which illustrates the difficulty of fire-proofing thin materials. The paper analyzed 13.6% zinc and 3.1% chlorine.

Paper similarly treated with zinc chloride in pulp form was filtered and pressed into thick pieces of paper as above. These were treated with 2 mols of ammonia per mol of zinc retained in the paper. The fire resistance was an E. The product analyzed 14.6% zinc and 2.8% chlorine.

## 16

## EXAMPLE XVI

A piece of wet strength paper toweling (Scott Paper Co.) was soaked in a water solution containing 50% zinc chloride and dewatered to 200% pick-up. It was then placed in a covered container with 2 mols of gaseous ethylene oxide per mol of zinc chloride retained by the paper toweling, for 16 hours, at room temperature. The paper was then dried at 70° C. Its fire resistance was E. The paper analyzed 31.6% zinc and 7.6% chlorine. After rinsing and redrying at 70° C., the fire resistance was still E. After washing at 60° C., in an agitator-type washing machine with a .5% detergent solution as in Example I, the fire resistance was G—.

The treated paper was noticeably whiter and more opaque than the original paper. The tear resistance of the treated paper appeared to be superior to that of the untreated paper.

20

## EXAMPLE XVII

A piece of five ounce cotton twill was treated with zinc chloride and ethylene oxide as in Example IX. Its analysis, after it had been rinsed and dried, showed 24.9% zinc and 5.6% chlorine. The cloth was then dry cleaned by tumbling, in five minute cycles, in trichloroethylene solution. At the end of each five minute cycle it was air dried, then covered with a moistened cloth and pressed dry with a hot iron. After twenty cleaning cycles, the cloth had a fire resistance of E. It analyzed 21.3% zinc and 5.3% chlorine, which shows that organic solutions such as those used in dry cleaning do not remove the basic zinc chloride.

35

## EXAMPLE XVIII

A piece of five ounce cotton twill treated with zinc chloride as in the first step in Example IX was placed in a solution of ammonia in trichloroethylene. The amount of ammonia in the trichloroethylene solution was in the proportion of 2 mols of ammonia to 1 mol of zinc chloride contained in the cloth. After 20 hours at room temperature, the cloth was removed, dried, and rinsed. The cloth analyzed 15.6% zinc and 14.1% chlorine. Its fire resistance after rinsing was E.

45

## EXAMPLE XIX

A piece of five ounce cotton twill was treated with zinc chloride solution as in the first step of Example IX, and then placed in a solution of ethylene oxide in trichloroethylene. The ethylene oxide dissolved was equivalent to 2 mols of ethylene oxide to one of zinc chloride in the cloth. The cloth was removed from the solution after 20 hours, air dried, rinsed, and dried again. The cloth analyzed 20.7% of zinc and 4.0% chlorine and showed a fire resistance after rinsing of E. After a wash in a .5% detergent solution as in Example I, at 60° C., the fire resistance was E. A two hour period of exposure to the ethylene oxide produced a cloth containing 13.1% zinc and 2.7% chlorine.

55

## EXAMPLE XX

A piece of five ounce cotton twill was soaked in a water solution containing 30% zinc chloride and 10% magnesium chloride for 15 minutes at 25-30° C. The excess of water was removed to give 200% pick-up. The piece was placed in a covered container and exposed to the equivalent of 2 mols of ethylene oxide per mol of zinc chloride, for 16 hours at room temperature. The cloth was then air dried for 10 minutes and subsequently oven dried for 30 minutes at 70° C. The cloth analyzed 4.5% magnesium, 7.0% zinc, and 9.2% chlorine. The fire resistance of the cloth was E, but its resistance to washing was poor.

It may be observed from the examples that the fire

resistance of the fabric and permanence of the treatment are not altogether dependent upon the amounts of zinc and chlorine retained by the fabric, but are also dependent upon the manner in which the fabric is impregnated.

The optimum amount of retained zinc for cloth which is to remain soft is 15-25%. In order to obtain this range, approximately a 200% wet pick-up of 40% zinc chloride solution is desirable, whereas if a 60% zinc chloride solution is used, a 140% wet pick-up is satisfactory.

When the concentration of zinc chloride solution exceeds about 65%, the zinc chloride begins to react with cotton cloth to "parchmentize" or "mercerize" it. At a concentration of 70-75% zinc chloride, the reaction is strong. When this reacted cloth is treated with ethylene oxide, and rinsed, the cloth is stiff and harsh, but its fire resistance is excellent, even after many washings. In treating cellulosic fabric with these highly concentrated solutions of zinc chloride, it may be found desirable to apply the solution hot, so as to reduce the viscosity of the solution, or to spray the cloth and immediately to pass it through rollers, depending upon the amount of parchmentizing and impregnation required. The following example is illustrative of this heavy treatment.

#### EXAMPLE XXI

A piece of cotton twill was soaked in 75% aqueous zinc chloride solution for 30 minutes at room temperature. The wet pick-up was reduced to approximately 350%. The cloth was treated with 2 mol equivalent of ethylene oxide in a closed container for 16-20 hours.

The cloth was rinsed and dried. It analyzed 34.8% zinc and 9.5% chlorine. The fire resistance was E.

After washing, 20 cycles in 0.5% Orvus Granules at 60° C., the fire resistance was E-. The cloth analyzed 32.1% zinc and 4.0% chlorine.

The uses to which fabric treated in accordance with the process of this invention may be put are manifold. For example, clothing, tents, tarpaulins, curtains, carpets, rope, fishnets, and the like may be rendered fire resistant and cloth and paper, increasingly opaque. Heavy cloth, heavily treated, may be used for welders' curtains and fire walls of buildings. Such cloth may be suspended over potentially dangerous areas, to be dropped in case of fire to smother the flames. In such applications, the cloth may be reinforced with glass fibers, metallic threads, asbestos fibers or the like.

All pieces of wool cloth impregnated with basic zinc chloride in accordance with this invention, have been markedly intumescent.

Thus it can be seen that a two step process is provided by which a substantially pure deposit of a coprecipitate of zinc hydroxide and a normally water soluble zinc salt is formed in situ in the pores of porous material and in and on the fibers of fibrous material in such a way that the deposit strongly resists leaching or dislodgement, and that the treated materials themselves are unique.

Having thus described the invention, what is claimed and desired to be secured by Letters Patent is:

1. The process of treating cellulosic material comprising impregnating the material, in separate steps, with a solution of a water soluble zinc salt and with a reactant which produces, with a portion of said water soluble zinc salt, zinc hydroxide, and co-precipitating the zinc hydroxide and residual water soluble zinc salt, in the form of water-insoluble basic zinc salt, in situ.

2. The process of treating cellulosic material comprising first impregnating the material with a solution of water soluble zinc salt, then impregnating said material with a basic material which produces, with a portion of said water soluble zinc salt, zinc hydroxide, and co-precipitating the zinc hydroxide and residual water soluble zinc salt, in the form of water insoluble basic zinc salt, in situ.

3. The process of treating a fabric, comprising wetting the fibers of said fabric with an impregnant solution con-

taining a water-soluble zinc salt, then thereafter introducing into the impregnated fabric a reactant, in a medium by which the zinc salt is not leached or dislodged, capable of reacting with the impregnant to co-precipitate therefrom zinc hydroxide and the said water-soluble zinc salt, and drying the said fabric.

4. Fabric containing zinc hydroxide and a water-soluble zinc salt co-precipitated in accordance with the process of claim 3.

5. The process of claim 3 wherein the reactant is a gaseous substance taken from the group consisting of ammonia and ethylene oxide.

6. The process of claim 3 wherein the reactant is an alkylene oxide.

7. The process of claim 3 wherein free solution is removed from the fabric after the fibers of the fabric are wetted, and the reactant is supplied in solution in an organic solvent in which the water-soluble zinc salt is substantially insoluble.

8. The process of claim 3 wherein the solution containing a water-soluble zinc salt also contains an organic fabric-treating material soluble in the water-soluble zinc salt solution and precipitated from solution with the basic zinc salt.

9. The process of treating wood comprising impregnating the wood with a water-soluble zinc salt taken from the group consisting of zinc chloride, zinc sulfate, chromated zinc chloride and chromated zinc sulfate, and subsequently impregnating the wood with an amount of a basic material sufficient to co-precipitate zinc hydroxide and the said water soluble zinc salt in situ in the wood.

10. The process of treating wood in which there are pores, comprising filling pores of the wood with a concentrated solution of a water-soluble zinc salt taken from the group consisting of zinc chloride, zinc sulfate, chromated zinc chloride and chromated zinc sulfate, at least partly evacuating the said pores of free solution, filling said pores with a basic material, and co-precipitating zinc hydroxide and the said water soluble zinc salt on the walls of said pores.

11. The process of treating wood comprising impregnating wood with a basic material, subsequently impregnating the wood with sufficient of a water-soluble zinc salt taken from the group consisting of zinc chloride, zinc sulfate, chromated zinc chloride and chromated zinc sulfate, to co-precipitate zinc hydroxide and the said water soluble zinc salt in situ in the wood and to produce a pH in the impregnated wood of less than 7.

12. The process of treating wood comprising impregnating the wood with zinc chloride, subsequently impregnating the wood with a solution containing sufficient ammonia to co-precipitate zinc hydroxide and the said zinc chloride in situ in the wood.

13. The process of claim 12 wherein the solution of ammonia contains zinc chloride.

14. The process of claim 12 wherein the solution of ammonia contains basic zinc chloride.

15. The process of treating wood comprising impregnating the wood with zinc sulfate and subsequently impregnating the wood with a basic material and co-precipitating zinc hydroxide and zinc sulfate as basic zinc sulfate.

16. The process of claim 9 wherein the basic material contains an anion taken from the group consisting of chloride, sulfate, bromide, phosphate, arsenite, arsenate, and borate.

17. The process of treating wood comprising impregnating wood with a solution of zinc chloride, subsequently impregnating the wood with ethylene oxide and precipitating basic zinc chloride in situ in the wood.

18. The process of producing fire resistant wood having low electrical conductivity, comprising leaching the wood with water to remove water-soluble salts, impregnating the wood with zinc chloride, impregnating the wood with ethylene oxide, precipitating basic zinc chloride in situ

in the wood, drying the wood, and evaporating the volatile reaction products of the zinc chloride and ethylene oxide.

19. The process of claim 9 wherein one of the impregnants contains an arsenic compound, which is precipitated with the basic zinc sulfate.

20. Wood treated in accordance with the process of claim 18, having low electrical conductivity, from which water-soluble salts have been leached, which contains practically pure basic zinc chloride and which has a pH of less than 7.

## References Cited in the file of this patent

## UNITED STATES PATENTS

|    |           |              |                |
|----|-----------|--------------|----------------|
| 5  | 831,450   | Lowry        | Sept. 18, 1906 |
|    | 1,318,523 | Arent et al. | Oct. 14, 1919  |
|    | 1,337,380 | Alexander    | Apr. 20, 1920  |
|    | 1,846,185 | Cline et al. | Feb. 23, 1932  |
|    | 2,097,509 | Boller       | Nov. 2, 1937   |
| 10 | 2,637,691 | Pershall     | May 5, 1953    |
|    | 2,769,730 | Sak Ornbut   | Nov. 6, 1956   |